

Oct. 24, 1933.

W. WHEELER

1,932,057

RECORD CORE

Filed Oct. 3, 1930

3 Sheets-Sheet 1



Fig. 4.



Fig. 5.



Fig. 6.



Fig. 1.



Fig. 2.



Fig. 3.

William Wheeler  
 Inventor  
 By his Attorney  
 Frederick W. Barker

106-80

CROSS REFERENCE

SEARCHED

Oct. 24, 1933.

W. WHEELER

1,932,057

RECORD CORE

Filed Oct. 3, 1930

3 Sheets-Sheet 2



william wheeler  
By his Attorney  
Frederick W. Barker

106-80

CROSS REFERENCE

EXAMINER

Oct. 24, 1933.

W. WHEELER

1,932,057

RECORD CORE

Filed Oct. 3, 1930

3 Sheets-Sheet 3



Fig. 9.

Inventor

William Wheeler

By his Attorney

Frederick W. Parker

XR

## UNITED STATES PATENT OFFICE

1,932,057

## RECORD CORE

William Wheeler, Brooklyn, N. Y.

Application October 3, 1930. Serial No. 486,204

16 Claims. (Cl. 274—42) ✓

This invention relates to records for phonographs, talking pictures and broadcasting, and my improvements are directed to a process of producing the cores of records from fibre board, whereby said cores will be free from any tendency to warp or become distorted.

The inexpensive and light weight characteristics of fibre board render it desirable as a core for records, but heretofore no satisfactory treatment for this material has been known that enables disks thereof to maintain a permanent flat condition, such as is necessary for record making purposes.

Therefore my invention consists in treating disks of fibre board by certain steps in a process that have the effect of destroying the life in the fibres to render them inert, and in compacting the board.

The steps of the process comprise:

20 (1) Producing a disk of fibre board, as by stamping it from a sheet and providing the central orifice therein; (2) chamfering the disk edges; (3) rotating the disk at an outward portion of its diameter between opposed pressure rollers to have the effect of expanding the disk diameter radially; then reducing the thickness of the disk at its central portion, as by grinding away the surface material, at both sides, within a limited radius; then subjecting the chamfered 25 peripheral portion of the disk to treatment by a quick drying gum solution, to seal the edge; then passing numerous high tension, electrical discharges through the disk to render it foraminous and burn the tension fibres, thereby taking the 30 life out of the material. The next step consists in coating the disk with a suitable fluid composition of vegetable origin and, while the composition is moist, there is dusted or sifted thereon a coating composed of gum and zinc oxide.

40 Record cores thus produced may have placed thereon disks of paper (which may bear pictures or other surface representations, which previously have been perforated by numerous high tension, electrical discharges passed therethrough; and 45 the cores, with their paper faces, are then subjected to moulding pressure at suitable temperature which causes the surfacing material on the core to penetrate the perforations in the paper disks, and to constitute record surfaces with the 50 moulded sound recording lines imparted thereto by the matrix.

Other features and advantages of my invention will hereinafter appear.

In the drawings:

55 Figure 1 is a plan view of a disk that has been

stamped or otherwise formed out of a sheet of fibre board, with a central hole therein.

Fig. 2 is a central sectional view of Fig. 1.

Fig. 3 is a like section showing the peripheral edges of the disk to have been chamfered.

Fig. 4 shows a disk undergoing pressure between rollers.

Fig. 5 is a plan view of a disk with its edges chamfered and its centre recessed.

Fig. 6 is a section through the centre of Fig. 5.

Fig. 7 shows a disk undergoing treatment at its chamfered edges in a sealing bath.

Fig. 8 is a side elevation of an apparatus with which the disks are perforated by electrical discharges while sliding by gravity into a surfacing bath.

Fig. 9 is a plan view of Fig. 8.

The basis for my improved record core is fibre board, by which is meant cardboard, pasteboard, 75 or other board composed of fibrous material. Disks, such as indicated at 1, are cut or stamped from this material and the usual stud or pin hole 2 for a record may be produced in the same operation. As another step in the process, the opposite peripheral edges of the disk are beveled down, or chamfered, as at 3, giving the peripheral portion of the disk a wedge-like appearance. This is for a purpose which will be referred to hereinafter. Also the disk, in an outward annulus over its area, indicated at 4, is subjected 80 to pressure between opposed rollers, each as are shown at 5, 5 in Fig. 4. This is for the purpose of expanding the material of the disk at the outward annulus 4 thereof, to compensate for the moulding pressure that is subsequently applied. 85

Still another step in producing the core consists in recessing the disk, at both sides, in the central, circular area 6, the recesses being formed as by grinding out the material to a desirable 90 depth in such area. By thus recessing or depressing the central area, the disk material in the region thus represented is relieved from the hydraulic or other heavy moulding pressure when that is applied in the formation of the record, in consequence whereof the surrounding portion of the device which is to bear the music, or other sound recording lines, becomes thereby more efficiently impressed. 95

In Figs. 7 there appears a shallow bath 7 which contains manila gum dissolved in acetone 105 or acetic ether in proportions which may be approximately 1 lb. manila gum to 2 gals. acetone or acetic ether. The disk (or a number thereof) is rotated with its chamfered peripheral portion entered in this solution, for impregna- 110

tion thereby, the chamfered edges being more readily absorbent than the disk surfaces would be. The solution being highly volatile, dries instantly and seals the disk edge interstices exposed by the chamfering, the gum also according a degree of stiffness to the chamfered periphery.

Still another step in my improved process of making records consists in subjecting the disks to the influence of high tension, electrical discharges, for the purpose of perforating the disks with numerous tiny orifices, produced by the passage of electric sparks through the disk material, burning the fibres thereof and rendering the material inert and incapable of warping or distortion.

For this purpose I employ the apparatus shown in Figs. 8 and 9, said apparatus comprising a metallic plate 8 which is supported in an inclined position as by the standards 9, 10, the standard 10, at the low end of plate 8 being represented as extending from a vessel 11, which is adapted to contain a liquid composition, constituting a bath. The angle at which plate 8 is set may be sufficiently steep to enable the disks, when placed thereon, to slide down said plate by gravity, and the vessel 11 is so related to the lower end of plate 8, that the disks will plunge into the bath upon leaving the plate. A plate 12, of insulation material, is placed over plate 8, in spaced parallelism therewith, and is supported as by screws 13, whereby also the spacing between plates 8, 12 may be adjusted. Numerous electrodes, 14, are carried by insulation plate 12, the electrodes for example being in the form of ordinary wood screws or machine screws that are threaded through plate 12, with their ends opposed to plate 8 and distanced from said plate sufficiently to enable a high tension, static current electrical discharge to pass between said electrodes and said plate 8.

Electrical current may be supplied from a power source as by the circuit wires 15, through the intermediary of high tension coils 16, whose secondary windings are shown as including in parallel respective groups of the electrodes 14.

The arbitrary arrangement of the electrodes 14, indicated in Fig. 8, as carried by insulation plate 12, shows groups of the screws disposed in a succession of transverse areas, whereby each disk, in sliding down plate 8, passes between a large number of electrodes and the plate 8, so that each disk in transit becomes penetrated by numerous electrical discharges.

The bath in vessel 11 is composed of approximately one part of rice flour dissolved in two parts of water glass. Also a proportion of Manila gum is added to the bath, the quantity thereof being from 10% to 50% of the combined rice flour and water glass mixture. The consistency of the mixture is affected by the proportion of manila gum used.

Congo gum can be used either instead of the manila gum or in conjunction therewith. Also rosin can be used as a substitute for the gums provided a sufficient proportion of rice flour be used to render the product hard.

It is to be understood that I intend water glass to equally comprehend a suitable silica solution, and for rice flour other suitable vegetable flour may be substituted. Or, in place of flour, either lamp black or rotten stone may be employed. But I have been able to obtain the best results by using rice flour.

75 The disks that have been immersed in the bath

are at once removed therefrom and are found to have received a surfacing of the bath composition which has been described. Before this surfacing dries the disks have sifted thereon a powdered mixture of manila gum and zinc oxide, the zinc oxide being in proportions of from 10% to 50% of the manila gum. This powdered mixture adheres to the surfacing composition, and the disk, thus treated, is in readiness to have a paper record sheet placed thereon.

This record sheet is a disk of paper which may have printed or otherwise imposed thereon a picture or other representation.

Said disk of paper may be slightly larger than the core disk and has been subjected to the electrical perforating process that has been described with respect to the core disk, so that it also is foraminous.

Said disk of paper is placed upon the treated core disk and then both disks are subjected to hydraulic or other suitable pressure of about 80 tons, at a temperature of from 150 to 300 degrees F. at which pressure and temperature the record lines are produced in the paper disk from the matrix, the heat and pressure causing the surfacing composition from the core disk to penetrate the paper disk through the perforations therein, and to constitute the record surface. Also in the mould the edge material of the slightly larger diameter of the paper disk folds over the peripheral edge of the disk core, binding said edge and giving a finished appearance to the record.

It is to be understood that the addition of the paper disk upon the record core is not absolutely necessary for the production of a sound producing record, because in some instances the record core, alone, and without the surfacing paper disk, can be subjected to the pressure under heat in the matrix for the creation of the sound producing lines thereon.

Or the record core can, if desired, be surfaced with shellac as its surfacing material.

Instead of the hereinbefore recited liquid composition of rice flour, water glass and manila gum as the surfacing material for the record cores I may, in some instances, employ a composition consisting of approximately equal proportions of rice flour and a solution of gum arabic, with from 10% to 50% of manila gum. The manila gum, according to the proportion thereof employed, affects the flowing quality of the composition; also hardening its surface, and rendering it waterproof.

This substitute composition may also, before drying, have a mixture of powdered manila gum and zinc oxide dusted over its surface. With a fibre board disk rendered foraminous by the penetration thereof with numerous high tension, electrical discharges, said disk being coated with a surfacing composition such as has been described, and then subjected to heat and pressure for the purpose of impressing the record lines thereon, it is found that the tiny perforations through the disk permit the liberation under the pressure of occluded gases which otherwise might cause blistering of the record surface to occur.

Variations within the spirit and scope of my invention are equally comprehended by the foregoing disclosure.

I claim:

1. The method of making record cores which consists in producing disks from fibre board, applying moderate pressure to an annular, outward portion of the disks, recessing the central por-

80

85

90

95

100

105

110

115

120

125

130

135

140

145

150

tions of said disks, and burning perforations through said disks to kill the fibre tension.

2. The method of making record cores which consists in producing disks from fibre board, 5 chamfering the edges of the disks, applying moderate pressure to an annular, outward portion of the disks, recessing the central portions of said disks, treating the chamfered edges with a volatile gum solution, and burning perforations 10 through said disks to kill the fibre tension.

3. The method of making record cores which consists in producing disks from fibre board, applying moderate pressure to an annular, outward portion of the disks, recessing the central portions of said disks, burning perforations through 15 said disks to kill the fibre tension, and applying a surfacing composition to said disks.

4. The method of making record cores which consists in producing disks from fibre board, 20 chamfering the edges of the disks, applying moderate pressure to an annular, outward portion of the disks, recessing the central portions of said disks, treating the chamfered edges with a volatile gum solution, burning perforations through 25 said disks to kill the fibre tension, and applying a surfacing composition to said disks.

5. The method of making records which consists in producing disks from fibre board, killing 30 the tension of the fibres thereof, coating the surfaces of the disks with a composition of vegetable flour, water glass and gum, and producing the record lines under heat and pressure.

6. The method of making records which consists in producing disks from fibre board, killing 35 the tension of the fibres thereof, coating the surfaces of the disks with a composition of rice flour, water glass and manila gum, and producing the record lines under heat and pressure.

7. The method of making records which consists in producing disks from fibre board, killing 40 the tension of the fibres thereof, coating the surfaces of the disks with a composition of vegetable flour, water glass and gum, dusting the composition while moist with powdered gum and zinc 45 oxide, placing sheets of foraminous paper on the surfaced disks, and producing the record lines under heat and pressure.

8. The method of making records which consists in producing disks from fibre board, killing 50 the tension of the fibres thereof, coating the surfaces of the disks with a composition of vegetable

flour, water glass and gum, dusting the composition while moist with powdered gum and zinc oxide, placing sheets of foraminous paper, which may bear pictorial representations, on the surfaced disks, and producing the record lines under heat and pressure.

9. A record core comprising a disk of fibre board that is provided with numerous burnt-in 80 perforations.

10. A record core comprising a disk of fibre board whose edges are chamfered and sealed with gum, said disk having centrally disposed recesses at its sides, and having a compacted outward annular portion.

11. A record core comprising a disk of fibre board that is provided with numerous burnt-in 90 perforations, said disk bearing a surfacing composition of vegetable flour, water glass and manila gum.

12. A record comprising a disk of fibre board 95 that is provided with numerous burnt-in perforations, said disk bearing a surfacing composition of vegetable flour, water glass and manila gum, and record lines impressed therein.

13. A record comprising a disk of fibre board 100 that is provided with numerous burnt-in perforations, said disk bearing a surfacing composition of vegetable flour, water glass and manila gum, a foraminous paper disk on said composition, and record lines impressed upon the composition extruded through said paper disk.

14. A record comprising a disk of fibre board 105 that is provided with numerous burnt-in perforations, said disk bearing a surfacing composition of vegetable flour, water glass and manila gum, 110 a foraminous paper disk, bearing a pictorial representation, on said composition, and record lines impressed upon the composition extruded through said paper disk.

15. A record surfacing composition consisting 115 of rice flour water glass and manila gum.

16. The method of making records which consists in producing disks from fibre board, passing numerous high-tension electrical discharges 120 through the disks to kill the tension of the fibres, coating the surfaces of the disks with a composition of vegetable flour, water glass and gum, and producing the record lines under heat and pressure.

WILLIAM WHEELER. 125